# EUROPEAN PATENT SPECIFICATION

(11) **EP 0 049 033 B1**
(45) Date of publication and mention of the grant of the patent: **21.11.1985**
(21) Application number: 81303337.0
(22) Date of filing: 21.07.1981
(51) Int. Cl.: C22C 38/26

(54) **Brazeable ferritic stainless steel, method of using same and article formed therefrom**
Hartlötbarer ferritischer rostfreier Stahl, Verfahren zur Verwendung dieses Stahls sowie aus diesem Stahl hergestellte Gegenstände
Acier ferritique inoxydable pouvant être brasé, procédé d'utilisation de cet acier et articles faits en cet acier

(30) Priority: 08.08.1980 US 176324
(43) Date of publication of application: 07.04.1982
(73) Proprietor: ALLEGHENY LUDLUM CORPORATION, Pittsburgh Pennsylvania 15222 (US)
(72) Inventor: Aggen, George, Sarver Pennsylvania 16055 (US); Borneman, Paul Richard, Sarver Pennsylvania 16055 (US)
(74) Representative: Sheader, Brian N.

## Description

The present invention relates to brazeable ferritic stainless steels and is particularly useful for ferritic stainless steel articles which are joined by brazing.

Ferritic stainless steels possess excellent mechanical properties and oxidation and general corrosion resistance at elevated temperatures. These steels are ideal for use as the structural members of heat exchangers, exhaust systems, chemical process vessels and the like which are exposed to high temperatures and stresses and corrosive environments. Fabrication of these articles frequently requires the joining of the ferritic stainless steel with either itself or with another dissimilar metal at sufficiently high temperatures for the joining method to be effective. Also, generally speaking, the steel must be joined in a temperature range exceeding the anticipated service temperature. Brazing is a widely practised method of joining metals involving temperatures of from 427°C (800°F) to the 1093°C-1149°C (2000°F-2100°F) range which are above the melting point of the brazing filler material but below the melting point of the base metal being joined. When the temperature of the brazing filler material is about the melting point, it becomes molten and wets the surface of the steel, and then flows by capillary action to fill a joint. Bonding results from the intimate contact produced by the dissolution of a small amount of the base metal in the molten filler metal.

Ferritic stainless steels to be joined at high temperatures contain low levels of carbon and small amounts of stabilizing elements for combining with carbon and nitrogen to maintain the ferritic phase and to maintain the oxidation and corrosion resistance of the steel. Stabilizing elements such as titanium, niobium or tantalum react with the carbon and nitrogen to prevent the formation and precipitation of chromium carbides and nitrides at grain boundaries and the simultaneous depletion of chromium in the surrounding areas. Stabilizing elements must be added in amounts exceeding the theoretical requirement to assure complete stabilization of carbon and nitrogen. Titanium has been the preferred stabilizing element because of its very strong affinity for carbon and nitrogen, its low atomic weight and its availability. Other stabilizing agents including niobium and tantalum have not been favoured because they are more expensive and less effective on a weight basis than titanium and also because they are accompanied by a tendency toward weld cracking problems.

Titanium stabilized ferritic steels known in the prior art (see e.g., Lula et al. United States Patent No. 3,250,611) cannot be readily brazed with filler materials such as oxygen-free copper and nickel base alloys. These steels form a non-wettable surface film which prevents proper bonding between the ferritic stainless steel base metal and the brazing filler material even when furance brazing under vacuum or in an inert atmosphere. The oxygen-free copper as a high temperature brazing filler metal does not penetrate this surface film. Nickel alloy high temperature brazing filler metals usually contain boron and silicon additions to penetrate the surface film. Although the steel wettability is improved, these nickel base materials will also penetrate the grain boundaries thereby causing intergranular attack of the base metal. In addition, brazing operations are not aided by increased temperatures or by increased brazing times because the high temperature range is beginning to affect the grain size of the steel and prolonged time tends to increase film resistance. For these reasons, brazing with copper is impossible and brazing with nickel base metals is not consistent enough to be of practical value from a quality assurance viewpoint. Thus copper clad ferritic stainless steels are used in brazing applications when the brazing temperature is to reach 1093°C-1149°C (2000°F-2100°F). In this process, the copper cladding is brazed rather than the steel.

The present invention relates to a stabilized ferritic stainless steel composition which is wettable by conventional brazing materials used at temperatures of from 1093°C-1149°C (2000°F-2100°F) in furnace brazing practices.

The present invention provides a ferritic stainless steel containing, by weight, 10.5% to 13.5% chromium, up to 0.03% carbon, up to 0.05% nitrogen, up to 0.10% aluminium, up to 0.12% titanium and at least one other stabilizing element selected from niobium and tantalum in accordance with the relationship: the balance being iron optionally including up to 1.25% molybdenum, up to 1 % manganese and up to 1 % silicon and incidental impurities.

Preferred nitrogen and aluminium levels are up to 0.03% and up to 0.020% respectively.

The presence of niobium, tantalum and titanium in accordance with this stabilization relationship are sufficient to effectively stabilize the interstitial elements in the steel without forming a non-wettable surface film. The niobium and tantalum are present as additions to the melt. Where niobium is a stabilising element, it may preferably be present in an amount up to 1.0%. When tantalum is a stabilizing element, it may preferably be present in an amount up to 1.8%. Titanium may be present in the scrap feed or added to the melt. The titanium is responsible for the nature of the film which becomes non-wettable when titanium is present in amounts greater than about 0.12%. Greater amounts of titanium could be tolerated and the effect of titanium on wettability could be neutralized if titanium compounds stable at brazing temperatures such as Ti0₂, TiS and TiN are permitted to form. However, oxygen, sulphur and nitrogen have an undesirable effect on other steel qualties and generally they will be kept as low as possible. From a brazing viewpoint it is preferable to have a composition free from titanium. For this reason the titanium is preferably present in an amount up to 0.01 % by weight and, most preferably, up to 0.005%. The steel may also contain up to 0.1 % aluminium, up to 1.25% molybdenum, up to 1% manganese and up to 1% silicon to enhance its mechanical and corrosion properties. Articles of this composition are wettable by fillers such as copper, nickel and their alloys and can be successfully furnace brazed according to conventional practices.

In some cases, however, it may be desirable to both weld and braze the same article. Therefore, titanium is tolerated in controlled amounts, i.e. from at least 0.001 % up to 0.12%, to prevent weld cracking while maintaining reasonable wettability during brazing operations. Larger amounts of titanium render the steel unbrazeable for practical purposes.

To illustrate the beneficial results of the invention specimens from sixteen laboratory heats and two commercial heats were tested for wettability. The composition of the laboratory heats and the commercial heats are identified in Table I as Nos. 1-16 and Nos. A and B respectively. Laboratory heats Nos. 1-6 and 14-16 are alloys in accordance with the present invention; laboratory heats 7-13 and the commercial heats A and B are included for purposes of comparison.

Samples from the laboratory heats were hot rolled to about 2.54 mm (0.100 inch) and cold rolled to 0.508 mm (0.020 inch). The commercial samples were also cold rolled to 0.508 mm (0.020 inch). The cold rolled samples were then annealed and pickled in accordance with standard practices. Circular specimens of 38 mm (12 inch) diameter were stamped from the cold rolled strips and tested for brazing wettability in a resistance heated cold wall vacuum furnace.

The test generally consisted of placing a brazing filler material on each specimen and heating the specimens and filler materials to the melting point of the filler material. The wettability of the specimens were evaluated according to the parameter "d²/h", where "d" is the average diameter of the drop in inches which formed on the surface of the specimen and "h" is the height of the drop in inches, wettability being proportional to the area covered by the drop and inversely proportional to the height of the drop.

Specimens of the heats were tested at 1121°C (2050°F) in conventional furnace atmospheres with oxygen-free copper as a brazing filler material. No flux was applied because this would be an uncommon practice in furnace brazing operations. Short 3.175 mm (0.125 inch) lengths of 0.254 mm (0.010 inch) diameter wire with square ends were placed on and at the centre of each specimen heated. In vacuum tests, the furnace was evacuated cold, heated to 565°C (1050°F), held at a vacuum of one micron of mercury (133.3 Pa) or less while heating to the brazing temperature. In inert gas tests, the furnace was evacuated cold, heated to 565°C (1050°F) held at a vacuum of one micron (133.3 Pa) or less while heating to 649°C (1200°F), pressurized with nitrogen to 1500 microns (2.10⁵Pa) and heated to the brazing temperature.

In the reducing atmosphere tests, the furnace was evacuated cold, heated to 565°C (1050°F), held at a vacuum of one micron (133.3 Pa) or less while heating to 649°C (1200°F), pressurized with dry hydrogen (having a dew point of less than -62°C 4-80°F) to a pressure of 300,000 microns (4.10' Pa) and heated to the brazing temperature. The wettability ratings (d²/h) of the specimens are shown in Table II. The letter "C" indicates that the specimen was completely wetted.

The wettability of the laboratory melted compositions can be compared with each other and with the prior art compositions of Heats A and B to determine the adverse effects of titanium. The prior art compositions are clearly non-wettable. The stabilized compositions of Heats 1-4 and 14-16 contain up to 0.005 wt% of titanium and exhibit superior wettability under all atmospheres. The effect of increasing amounts of titanium is most clearly shown by the compositions of Heats 5-7. The composition of Heat 5 contains 0.008 wt% titanium and has superior wettability characteristics under all atmospheres. The composition of Heat 6 contains 0.11 wt% titanium and has improived wettability characteristics under inert gas and vacuum atmospheres, however the adverse effect of titanium is evident in a reducing atmosphere. Heats 7-13 contain large amounts of titanium and have no better wettability characteristics than do the prior art compositions.

The difference in wettability between the specimens brazed with oxygen-free copper in a dry nitrogen atmosphere is seen from Figures 1 and 2. Figures 1 and 2 are the perspective and top views, respectively, of a brazing table supporting the specimens identified in Tables I and II. Specimens A and B are the commercial steels and illustrate the problem where the filler material does not wet the surface beyond the periphery of the molten drop. Similarly, specimens 7, 8, 9 and 10 are also not wetted by the filler material. Specimens 1, 2, 3 and 4 are completely wetted by the oxygen-free copper. Specimens 5 and 6, although containing increasing titanium concentrations of 0.008% and 0.11 % respectively, are clearly wetted by the copper beyond the periphery of the molten drop.

Specimens of the Heats were tested at 1093°C (2000°F) under vacuum conditions with a nickel alloy as a brazing filler material. In these tests nickel alloy powder (AWS BNi-2) was mixed with a plastic cement which vaporized completely before reaching 538°C (1000°F). The mixture was formed into pellets of approximately 4.7625 mm (0.1875 inch) diameter by 4.7625 mm (0.1875 inch) height and the pellets were placed on the specimens. The furnace was evacuated cold and heated to the brazing temperature. No flux was applied because this is uncommon practice in furnace brazing at high temperatures. The wettability ratings of the laboratory melted specimens are shown in Table III. The letter "C" indicates that the specimen was completely wetted.

The prior art compositions were not tested but they would have a rating approximating those of Heats 7 and 9 respectively in view of their titanium contents. The compositions of Heats 3, 5 and 14-16 all contain less than .01 wt% titanium and have superior wettability characteristics. The composition of Heat 6 contains 0.11 wt% titanium and has superior wettability characteristics in comparison to the other compositions containing 0.18 wt% (Heat 12) or more titanium (Heats 7 and 9).

## Claims

1. A brazeable ferritic stainless steel containing, by weight, 10.5% to 13.5% chromium, up to 0.03% carbon, up to 0.05% nitrogen, up to 0.10% aluminium, up to 0.12% titanium and at least one other stabilizing element selected from niobium and tantalum in an amount in accordance with the relationship: the balance being iron optionally including up to 1.25% molybdenum, up to 1% manganese and up to 1% silicon and incidental impurities.

2. A brazeable ferritic stainless steel according to claim 1, containing, by weight, up to 0.03% nitrogen and up to 0.020% aluminium.

3. A brazeable ferritic stainless steel according to claim 1 or claim 2, wherein the titanium is present in amounts up to 0.01%.

4. A brazeable ferritic stainless steel according to claim 1 or claim 2, wherein the titanium is present in amounts up to 0.005%.

5. A brazeable ferritic stainless steel according to any one of the preceding claims, wherein the titanium is present in amounts of at least 0.001 %.

6. A brazeable ferritic steel according to any one of the preceding claims, stabilized by niobium.

7. A brazeable ferritic steel according to claim 6, wherein the niobium is present in an amount up to 1.0%.

8. A brazeable ferritic steel according to any one of the preceding claims 1 to 5, stabilized by tantalum.

9. A brazeable ferritic steel according to claim 8, wherein the tantalum is present in an amount up to 1.8%.

10. A method of using the ferritic stainless steel of any one of the preceding claims, comprising brazing the steel.

11. A method of using the ferritic stainless steel of any one of claims 1 to 9 comprising brazing the steel with copper.

12. A brazed ferritic stainless steel article having the composition of the steel of any one of claims 1 to 9.

13. A ferritic stainless steel article having the composition of the steel of any one of claims 1 to 9, wherein the article is brazed with copper.

## Patentansprüche

1. Hartlötbarer ferritischer nichtrostender Stahl mit 10,5 bis 13,5 Gew.-% Chrom, bis zu 0,03 Gew.-% Kohlenstoff, bis zu 0,05 Gew.-% Stickstoff, bis zu 0,10 Gew.-% Aluminium, bis zu 0,12 Gew.-% Titan und wenigstens ein weiteres Stabilisierungselement in Form von Niob oder Tantal in einer Menge gemäß der Gleichung: wobei der Rest aus Eisen besteht und wahlweise bis zu 1,25 Gew.-% Molybdän, bis zu 1 Gew.-% Mangan und bis zu 1 Gew.-% Silizium und zufällige Verunreinigungen enthält.

2. Hartlötbarer ferritischer nichtrostender Stahl nach Anspruch 1, mit bis zu 0,03 Gew.-% Stickstoff und bis 0,020 Gew.-% Aluminium.

3. Hartlötbarer ferritischer nichtrostender Stahl nach Anspruch 1 oder 2, wobei das Titan in Mengen bis zu 0,01% vorliegt.

4. Hartlötbarer ferritischer nichtrostender Stahl nach Anspruch 1 oder 2, wobei das Titan in Mengen bis zum 0,005% vorliegt.

5. Hartlötbarer ferritischer nichtrostender Stahl nach einem der vorhergehenden Ansprüche, wobei das Titan in Mengen von wenigstens 0,001% vorliegt.

6. Hartlötbarer ferritischer Stahl nach einem der vorhergehenden Ansprüche, stabilisiert durch Niob.

7. Hartlötbarer ferritischer Stahl nach Anspruch 6, wobei das Niob in einer Menge bis 1,0% vorliegt.

8. Hartlötbarer ferritischer Stahl nach einem der vorhergehenden Ansprüche 1 bis 5, stabilisiert durch Tantal.

9. Hartlötbarer ferritischer Stahl nach Anspruch 8, wobei das Tantal in einer Menge bis 1,8% vorliegt.

10. Verfahren zur Verwendung des ferritischen nichtrostenden Stahls nach einem der vorhergehenden Ansprüche, gekennzeichnet durch Hartlöten des Stahls.

11. Verfahren zur Verwendung des ferritischen nichtrostenden Stahls nach einem der Ansprüche 1 bis 9, gekennzeichnet durch Hartlöten des Stahls mit Kupfer.

12. Gegenstand aus hartgelötetem ferritischem nichtrostenden Stahl mit der Zusammensetzung des Stahls nach einem der Ansprüche 1 bis 9.

13. Gegenstand aus ferritischem nichtrostendem Stahl mit der Zusammensetzung des Stahsl nach einem der Ansprüche 1 bis 9, wobei der Gegenstand mit Kupfer hartgelötet ist.

## Revendications

1. Acier inoxydable ferritique à braser caractérisé en ce qu'il contient, en poids, 10,5 à 13,5% de chrome, jusqu'à 0,03% de carbone, jusqu'à 0,05% d'azote, jusqu'à 0,10% d'aluminium, jusqu'à 0,12% de titane et au moins un autre élément stabilisant choisi entre le niobium et le tantale en une quantité vérifiant la relation: le reste étant du fer et contenant éventuellement jusqu'à 1,25% de molybdène, jusqu'à 1 % de manganèse et jusqu'à 1% de silicium et des impuretés accidentelles.

2. Acier inoxydable ferritique à braser selon la revendication 1, caractérisé en ce qu'il contient, en poids, jusqu'à 0,03% d'azote et jusqu'à 0,020% d'aluminium.

3. Acier inoxydable ferritique à braser selon la revendication 1 ou 2, caractérisé en ce que le titane est présent en des quantités allant jusqu'à 0,01%.

4. Acier inoxydable ferritique à braser selon la revendication 1 ou 2, caractérisé en ce que le titane est présent en des quantités allant jusqu'à 0,005%.

5. Acier inoxydable ferritique à braser selon l'une quelconque des revendications précédentes, caractérisé en ce que le titane est présent en quantités d'au moins 0,001%.

6. Acier ferritique à braser selon l'une quelconque des revendications précédentes, caractérisé en ce qu'il est stabilisé par le niobium.

7. Acier ferritique à braser selon la revendication 6, caractérisé en ce que le niobium est présent en ur. quantité allant jusqu'à 1,0%.

8. Acier ferritique à braser selon l'une quelconque des revendications 1 à 5, caractérisé en ce qu'il est stabilisé par le tantale.

9. Acier ferritique à braser selon la revendication 8, caractérisé en ce que le tantale est présent en une quantité allant jusqu'à 1,8%.

10. Technique utilisant l'acier inoxydable ferritique selon l'une quelconque des revendications précédentes, caractérisée en ce qu'elle comprend le brasage de l'acier.

11. Technique utilisant l'acier inoxydable ferritique selon l'une quelconque des revendications 1 à 9, caractérisée en ce qu'elle comprend le brasage de l'acier avec du cuivre.

12. Article en acier inoxydable ferritique à braser caractérisé en ce qu'il a la composition de l'acier selon l'une quelconque des revendications 1 à 9.

13. Article en acier inoxydable ferritique ayant la composition de l'acier selon l'une quelconque des revendications 1 à 9, caractérisé en ce que l'article est brasé avec du cuivre.
